

Nov. 24, 1931.

L. BRADLEY ET AL

1,833,313

## TREATMENT OF RESIDUAL LIQUORS.

Filed Jan. 14, 1924



Linn Bradley  
E. P. McKee

BY  
Pennie Davis Marvin Edwards  
ATTORNEYS

## UNITED STATES PATENT OFFICE

LINN BRADLEY, OF MONTCLAIR, NEW JERSEY, AND EDWARD P. MCKEEFE, OF NEW YORK, N. Y., ASSIGNEES TO BRADLEY MCKEEFE CORPORATION, A CORPORATION OF NEW YORK

## TREATMENT OF RESIDUAL LIQUORS

Application filed January 14, 1924. Serial No. 686,137.

This invention relates to improvements in the manufacture of pulp from wood with a cooking liquor containing essentially sodium sulfite, either alone or admixed with caustic soda, or with excess sulfur dioxide. More particularly it relates to the treatment of residual liquors from such processes.

In our prior application, Serial No. 481,147, filed June 28, 1921, we have described an improved method of pulp manufacture in which the pulp making operation is carried out with a cooking liquor containing essentially normal sodium sulfite, either with or without the addition of small amounts of caustic soda. In our prior application Serial No. 535,034, filed February 28, 1922, we have described another method of pulp manufacture in which the cooking liquor employed is made up essentially of caustic soda and sodium sulfite, with the caustic soda in predominating amount. In our prior application Serial No. 665,224 filed September 27, 1923 we have described still another method of pulp manufacture in which the cooking liquor is made up essentially of sodium sulfite with excess sulfur dioxide, in excess of that required for the normal sodium sulfite.

The present invention relates to improvements in the processes of said prior applications, and particularly in the treatment of residual liquors from the digestion or cooking operations of said processes, for the regeneration of further amounts of cooking liquor for use in such processes. According to the present invention, the cooking or digestion operation and the regeneration or recovery operations may advantageously be carried out in apparatus constructed and intended for carrying out the sulfate process so-called.

In the sulfate process so-called the cooking liquor consists essentially of caustic soda and sodium sulfide. Varying amounts of sodium carbonate, sodium sulfate, and other sodium compounds may also be present, but they are generally considered to be inert in the process. Sodium sulfate or nitre cake is employed as the source of the sodium sulfide, and a considerable part of it is reduced to

sodium sulfide during the smelting operation.

The sulfate process is recognized as having certain objections and limitations. The residual liquor is difficult to handle during the concentrating, calcining and smelting operations. Furthermore, the sulfate process is so objectionable in the malodors given off that sulfate pulp mills should be located away from centers of large population. Where located in well populated territory, the resulting nuisance has been such that court action has been successfully invoked to prevent operation of the process.

The process of the present invention may utilize the plant and equipment of existing sulfate mills, especially when the cooking liquor as charged into the digesters is alkaline to litmus, but it avoids the nuisance produced by the objectionable odors of the sulfate process, or so greatly reduces the odors formed that it is accordingly well adapted for use in existing sulfate mills which are located near centers of population where operation of the sulfate process is prohibited, or which may hereafter be prohibited by court order.

In the practice of the present invention, we may employ the digester of the sulfate mill for carrying out the cooking operation, provided it possesses sufficient strength. We prefer to employ digesters capable of operating at as high as 160 pounds pressure per square inch, and where the cooking liquor is acid to litmus to have the digester lined to protect the shell. We employ as cooking liquor a solution containing essentially normal sodium sulfite ( $Na_2SO_3$ ), or sodium sulfite and caustic soda, or sodium sulfite and excess sulfur dioxide. By the term "excess sulfur dioxide" we mean the sulfur dioxide content over and above the amount required to form the normal sodium sulfite. The cooking liquor may contain some sodium sulfide and it may contain some sodium thiosulfate or other sodium sulfur compounds as well as other sodium compounds. But we have found that where thiosulfate, or other sodium compounds which contain loosely combined sulfur, are present in the cooking liquor,

objectionable odors are much less when the cooking liquor contains a preponderating amount of sodium sulfite than when such reagent is absent. Especially when sodium 5 thiosulfate is present in appreciable amount, sodium sulfite in amount sufficient to cook the wood overcomes the objectionable features which the thiosulfate would produce if used alone. Therefore in this invention the 10 cooking of wood to produce pulp does not result in the formation of the malodorous compounds characteristic of the sulfate process, or at least such compounds are formed in a less objectionable degree.

15 The residual liquors from the cooking operation, with neutralization of free acid content if any, may be treated, according to the present invention, in the evaporators, rotary furnaces and smelters of the sulfate 20 process mill; but this treatment of the residual liquors is distinguished in important respects from the treatment of the residual liquors of the sulfate process in the same apparatus and equipment.

25 The present invention, furthermore, when carried out in a sulfate mill, requires only moderate alterations in the equipment, or in added equipment, of such a sulfate mill, so that a sulfate mill can be utilized for carrying 30 out the improved process of the present invention with small expense for added equipment.

15 The process of the present invention varies somewhat with the composition of the cooking liquor employed. These distinctions, from the standpoint of the cooking operation, are referred to in our prior applications in which these respective processes are described. The cooking operations can be carried 40 out with cooking liquors of varying compositions, and upon different kinds of woods, as pointed out in said prior applications.

45 Insofar as the pulp making operation itself is concerned, the process of the present invention presents the same advantages as the processes of our said prior applications, and is of more or less general application to woods of various kinds, including woods which are not commonly regarded as pulp 50 woods at all. The present invention is thus applicable not only to the usual pulp woods such as spruce and poplar, but is applicable to short-fiber hard woods such for example as birches, beeches, maples, etc. and also to other 55 long-fibered conifers, such as jack-pine, tamarack, loblolly pine, hemlock, etc.

60 At the end of the cooking or digestion operation, the residual liquor will be of a different composition and character from the residual liquor of the sulfate process. Some of the residual liquor may be used over again in making up the cooking liquor for a successive cook. Where dense hard woods are employed, the composition of the residual 65 liquors will be somewhat different than when

coniferous woods such as for example jack-pine, are used. It is one advantage of the process that the residual liquor may already be concentrated to a considerable degree in the sense that it may contain relatively much more organic matter and much more sodium compounds per unit volume than the residual liquor from the sulfate process when the latter is operated exclusively with fresh liquor.

70 The residual liquor, according to the present invention, is subjected to evaporation, calcination and smelting, using evaporators, calcining furnaces and smelters which may be those of a sulfate mill. The process does not present the difficulties of concentration which the black liquor from a sulfate mill presents, and the liquor can be concentrated to a high degree in multiple effect evaporators before introduction into the calcining furnaces; although the residual liquor may in some cases 75 be produced directly of such a concentration that it can be fed directly to the calcining furnaces.

80 From the calciners, the black ash may be charged into the smelter, together with additional carbonaceous material if necessary, and there subjected to a smelting operation. This smelting operation is distinguished in important respects from the smelting operation of the sulfate process. The black ash is easier to smelt. The melt or smelt obtained from the smelter can be dissolved in water and treated for the production of further amounts of cooking liquor therefrom 85 without the use of lime.

86 The operations thus far described may be carried out in the existing equipment of a sulfate mill, although the operations differ in important respects from the corresponding operations of the sulfate process. In particular, the digestion, concentration, calcination and smelting operations are carried out with materials of a different character and with less objectionable odors than the sulfate process gives.

90 In the sulfate process, the melt from the smelter contains relatively large amounts of sodium sulfide, and this sulfide is employed in the further carrying out of the cooking process. In the process of the present invention, however, the melt from the smelter will usually contain only a relatively small amount of sodium sulfide. This amount may be so small that it can be utilized in the cooking liquor in the further carrying out of the process, in which case the cooking liquor will contain a small amount of sodium sulfide as well as a preponderating amount of sodium sulfite, or of sodium sulfite and caustic soda. It may also contain some sodium thiosulfate.

95 Where, however, the sodium sulfide is not desired in the cooking liquor or where the amount of sodium sulfide in the melt is larger than is desired in the cooking liquor, the solu-

tion of the melt may be treated for the conversion of the sodium sulfide into other compounds. The invention includes different methods of treatment of the solution for this purpose.

The addition of further amounts of sodium compounds to make up for losses in the process may take place at different stages of the process. Salt cake or niter cake for example can be added to the desired extent to the residual liquor before or after concentration and advantageously before calcination, or after calcination and before smelting, and in such case, the added sodium sulfate may be converted largely into sodium sulfide by the smelting operation, so that the solution of the melt will contain a correspondingly increased amount of sodium sulfide, which may be utilized in the cooking operation or which may be advantageously converted into sodium sulfite or other compounds by suitable treatment.

Instead of adding sodium sulfate or niter cake or salt cake to supply added amounts of sodium, sodium carbonate may be employed and may be added for example to the solution of the melt before it is subjected to further treatment.

One way of treating the solution of the recovered sodium compounds, after calcination and smelting, to convert sodium sulfide into other sodium compounds of the kind described, is to subject the solution to treatment with carbon dioxide in such manner that a carbonate of sodium is formed. Hydrogen sulfide which is given off may be burned to produce sulfur dioxide and this sulfur dioxide utilized to convert sodium carbonate into sodium sulfite. This hydrogen sulfide may be burned in the combustion chamber of a sulfur burner and thus mixed with sulfur dioxide gas resulting from the combustion of sulfur, and this sulfur dioxide can be used for treating the solution containing the sodium carbonate to convert the carbonate to the desired extent into sodium sulfite.

The liquor may be treated to free it from sodium sulfide, where such treatment is desired, and then treated with lime to convert the greater portion of the contained sodium carbonate into caustic soda, care being taken that the sodium sulfite that may be contained in the liquor is not converted to any large extent into caustic soda. The causticized liquor will then contain caustic soda together with more or less sodium sulfite, and it may also contain varying amounts of sodium carbonate, sodium sulfate, sodium thiosulfate, etc. The composition of the liquor can be regulated for example by adding sodium carbonate before causticizing where the amount of caustic soda is to be increased, or by adding further amounts of sodium sulfite, or by forming further amounts of sodium sulfite in the liquor. In this way a cooking liquor

can be regenerated containing essentially sodium sulfite or containing sodium sulfite and caustic soda. The regenerated solution can also, where desired, be admixed with residual liquor from the digesters in making up the proper volume and concentration of active chemicals to the desired point for use in the further carrying out of the cooking operation.

The process thus far described requires but little added equipment to that of a sulfate mill. A small sulfur burner, a simple absorption tower, and conversion tanks for converting the sodium sulfide into other sodium compounds constitute most of the added equipment necessary. The added reagents to make up for those lost in the process may be supplied by lime, sodium carbonate and the burning of sulfur, or in part by niter cake or salt cake.

Where sodium bisulfate is added to the residual liquor, this sodium bisulfate will react with reactive sodium compounds to form normal sodium sulfate. The solution containing sodium sulfate and other sodium compounds and organic matter may be evaporated and calcined in other apparatus than the vacuum evaporators and rotary kilns. For example, the liquor may be subjected to spray evaporation with hot gases or otherwise, and the resulting dried product then subjected to the smelting operation. Where the liquor itself does not contain sufficient reducing materials (e. g. carbon from decomposition), further amounts of carbonaceous materials may be added so that the sodium sulfate will be largely reduced to sodium sulfide, and so that the melt may contain sodium carbonate and sodium sulfide together with some sodium sulfite, sodium sulfate and other compounds.

The incineration or calcination of the dried residual liquor results in the destructive distillation of the material and the formation of valuable products which may be passed through a condenser to condense combustible liquids such as alcohols, acetone, etc. Such liquor can be utilized by blending with other ingredients such as gasoline, alcohol, benzene, acetylene, etc. for making motor fuel or other fuel compositions. The non-condensable gases from the incineration or destructive distillation can be utilized as fuel, for example, in drying or evaporating the residual liquor.

When the solution of the melt contains a considerable amount of sodium sulfide or polysulfides together with sodium carbonate, the treatment of this solution directly with sulfur dioxide gas will set free carbon dioxide and cause more or less of the sodium sulfide and polysulfides to be converted into sodium thiosulfate ( $Na_2S_2O_3$ ). If the solution contains a fairly high percentage of sulfide or polysulfides, this direct treatment

70

75

80

85

90

95

100

105

110

115

120

125

130

of the solution with sulfur dioxide will result in a solution containing a high proportion of thiosulfate. According to the process of another invention of ours we take advantage of this formation of thiosulfate in producing a cooking liquor for cooking broad leaved or deciduous woods to produce a special kind of pulp therefrom. We have found that the use of such a cooking liquor, 10 consisting primarily of thiosulfate, is of advantage as applied to broad leaved or deciduous woods for producing certain kinds of special pulp, and that the residual liquor from such pulp making operations can be 15 treated for the recovery of the thiosulfate for further use in the cooking operation. This thiosulfate process, however, forms the subject of a separate application and we do not claim the same herein.

20 Where it is desired to obtain wood pulp suitable for bleaching, we have found that it is desirable to avoid the presence of a proportionally large amount of thiosulfate in the cooking liquor, and that it is desirable 25 to treat the residual liquors so that the cooking liquor obtained therefrom will contain a proportionally large amount of sodium sulfite. By using sufficient sodium sulfite in the cooking liquor, and only a relatively 30 small amount of thiosulfate, or no thiosulfate at all, the formation of dark pulp difficult to bleach is prevented. If the amount of sodium sulfite in the cooking liquor is equal to around 30 to 50% of the bone dry 35 weight of the wood, a considerable amount of thiosulfate may be contained in the cooking liquor and a readily bleachable pulp nevertheless obtained.

Where the residual liquor from such a 40 cooking operation, in which some sodium thiosulfate is used, is evaporated, calcined in the presence of air, and subsequently smelted, the thiosulfate undergoes decomposition and some sulfur is eliminated from the cycle, 45 so that the recovered chemicals can be treated for the production of cooking liquor of suitable composition without objectionable up-building of thiosulfate in the cooking liquor.

By suitable treatment of the solution of 50 the melt, the formation of sodium thiosulfate from the sodium sulfide of the solution can be substantially prevented. For this purpose, the solution can advantageously be treated first with carbon dioxide to convert the sodium sulfide into carbonate or bicarbonate and liberate hydrogen sulfide. Carbon dioxide gas, preferably in highly concentrated condition, may thus be passed into 55 an absorption tower or tank containing the solution of the melt. By decomposing the sulfides in this way and removing the hydrogen sulfide liberated, the formation of thiosulfate upon subsequent treatment of the solution with sulfur dioxide, is substantially

avoided. By using relatively pure and concentrated carbon dioxide and a suitable tower or tank, a nearly pure and concentrated hydrogen sulfide gas is driven off from the top of the tower or tank. This hydrogen sulfide gas, accompanied by any unabsorbed carbon dioxide, can then be burned, for example, by introducing it into the combustion chamber of a sulfur burner, thereby burning the hydrogen sulfide to sulfur dioxide and water. The sulfur dioxide thus formed will admix with that from the sulfur burner and can be employed in the manufacture of sodium sulfite.

The sulfur dioxide from the sulfur burner, together with the added sulfur dioxide from the combustion of the hydrogen sulfide, may be absorbed in an absorption tower or tank in a solution of sodium sulfite which gradually increases in free acid content. The temperature and the percentage of free and combined sulfur dioxide can be controlled at will. By regulating the concentration and rate of flow of the liquor and gas through the absorption tower or tank, a liquor of the desired content of sulfur dioxide and of the desired ratio of free to combined sulfur dioxide can be obtained. This solution can then be fed into the bottom of a tank containing a solution of sodium carbonate or bicarbonate or admixture thereof, with thorough agitation, and with the resulting setting free of carbon dioxide and the formation of a corresponding amount of sodium sulfite. This nearly pure carbon dioxide gas, or as much of it as necessary, can be used in treating the solution of the melt for converting the sodium sulfide into sodium carbonate and driving off hydrogen sulfide. The resulting solution, which may be substantially free from sodium sulfide, and containing a corresponding increased content of carbon dioxide, may be the solution to which the acid sulfite solution is added as above described. When the process is thus carried out, carbon dioxide may be used repeatedly and successively in reacting with the sodium sulfide to form sodium carbonate which is later decomposed with the acid sulfite solution to drive off the carbon dioxide again and form sodium sulfite.

The carbonated solution from the carbonating tower or tank, after the conversion of sodium sulfide into sodium carbonate is divided in such proportion as needed, part going to the sulfur dioxide absorption tower or tank and part going to make up the cooking liquor for the cooking operation. Where the cooking liquor is to contain essentially sodium sulfite ( $Na_2SO_3$ ) with only small amounts of other sodium salts or of caustic soda, the carbonated solution from the carbonating tower or tank may be neutralized with the acid sodium sulfite solution from the sulfur dioxide absorption tower or tank.

and a sufficient amount of the resulting solution employed in making up the cooking liquor.

Where the cooking liquor is to contain both sodium sulfite and caustic soda, a part of the sodium carbonate may be treated with lime and subjected to a regulated causticizing operation, and the proportions of caustic soda and sodium sulfite may be varied as desired.

It will be evident that where a cooking liquor which is acid in character is desired, for example, a cooking liquor containing an amount of sulfur dioxide greater than that corresponding to sodium sulfite and less than that corresponding to sodium bisulfite, the residual liquor can be subjected to a similar concentration, drying, calcining and smelting operation, and the solution of the melt can be treated in the manner above described, and the solutions so produced can be so combined that a cooking liquor containing the desired amounts of sulfur dioxide both free and combined can be obtained. Where for example an acid sodium sulfite cooking liquor is desired, the solution of sodium carbonate obtained by carbonating the solution of the melt to decompose the sodium sulfide and drive off hydrogen sulfide can be treated with sulfur dioxide or with a solution of sodium sulfite containing a sufficient excess of sulfur dioxide so that the resulting solution will be of the desired sulfur dioxide content as well as of the desired content of combined sulfur dioxide (calculated as  $\text{Na}_2\text{SO}_3$ ).

When the regenerated cooking liquor contains an excess of sulfur dioxide, in excess of that required for the normal sodium sulfite, an acid-proof lining may be required in the digester during the cooking operation, particularly where a large excess of sulfur dioxide is present. If the amount of excess sulfur dioxide is sufficiently small, an acid-proof lining may be unnecessary. The digester, when operated at higher pressures than those commonly employed in the sulfate process, should of course be of a stronger or reinforced construction which will permit the use of the high pressures desired.

The residual liquors from such an acid sulfite process in which an excess of sulfur dioxide is used over and above that required for the normal sodium sulfite can be treated in a similar manner to that above described, making use of the existing equipment of a sulfate mill, or using other suitable apparatus.

A flow sheet illustrating the recovery process above described is shown conventionally in the accompanying drawing. The residual liquor from the digester is subjected to evaporation in evaporators and then to incineration in incinerators, and to smelting, and the smelted product is then dissolved in dissolving tanks. The apparatus used in these op-

erations may be those of the sulfate process, as above described.

From the dissolving tanks, the liquor containing sodium carbonate and varying amounts of sodium sulfide, depending upon the composition of the residual liquor treated and the method of incineration, passes to one or the other of the two storage tanks indicated on the flow sheet as "CO<sub>2</sub> circulating tanks". From one or the other of these tanks the solution is circulated through the carbonating tower referred to on the blue print as "CO<sub>2</sub> tower". In this tower the solution is subjected to the action of carbon dioxide which acts upon the sodium sulfide to form a carbonate of sodium and to set free hydrogen sulfide. The hydrogen sulfide together with any unabsorbed carbon dioxide may be conveyed to the combustion chamber of the sulfur burner where the hydrogen sulfide is burned to form sulfur dioxide and water vapor.

When one of the tanks of liquor has been sufficiently carbonated it is pumped to one or the other of the two adjusting tanks where it is subjected to treatment with a solution of sodium bisulfite, or a solution of sodium sulfite containing a greater or smaller amount of SO<sub>2</sub> than corresponds to sodium bisulfite, preferably with introduction of the bisulfite solution at the bottom, and with gentle agitation. The action of this sodium bisulfite solution upon the sodium carbonate solution is to set free carbon dioxide in a relatively pure and concentrated state. The carbon dioxide may be collected in a gasometer from which a sufficient amount is supplied to the carbonating tower or tank while the surplus carbon dioxide can be passed to a compressor or otherwise utilized.

When one of the adjusting tanks has been neutralized and the carbonate decomposed the resulting solution of normal sodium sulfite can be in part conveyed to the digesters for use as a make-up liquor for further cooking operations, or its composition can be modified to give a cooking liquor of either acid or alkaline character. The remainder of the sodium sulfite solution from the adjusting tank may be conveyed to one or the other of the sulfur dioxide circulating tanks from which it is circulated through the sulfur dioxide absorption tower or tank to absorb a sulfur dioxide from the sulfur burner. By passing the hot gases from the sulfur burner through the absorption tower down which the sodium sulfite solution passes, the solution gradually increases in temperature, and in excess sulfur dioxide content. By regulating the concentration and rate of flow of liquor and gas, the amount of sulfur dioxide absorbed can be regulated and controlled until a solution corresponding to sodium bisulfite, or with greater or less sulfur dioxide content is obtained. The percentage of sulfur dioxide

absorbed can be controlled at will. This sodium bisulfite liquor can then be returned to one of the adjusting tanks or it can be in part employed in further cooking operation.

The sulfur dioxide from the sulfur burner together with the sulfur dioxide formed from the hydrogen sulfide is absorbed in the  $\text{SO}_2$  tower or tank while the inert gases (nitrogen and carbon dioxide) escape to the atmosphere.

The process of the flow sheet as described and illustrated is a self contained process in which the only added reagent is sulfur for the sulfur burner to supply additional sulfur dioxide; while the regenerative process gives a solution of either normal sodium sulfite or of sodium bisulfite or liquors of intermediate composition which can be used as such or further modified in the carrying out of the process. Carbon dioxide may be obtained as a by-product. Additional sodium to make up for losses in the process can be supplied in various ways. Soda ash or sodium carbonate can be added at any point prior to the treatment of the solution of sodium carbonate with the acid sodium sulfite solution. Sodium sulfate or niter cake, if used, should be added before the incineration so that it will be in part reduced to sodium sulfide during the smelting operation. The sodium sulfide so produced may be utilized for the formation of sodium carbonate, and the hydrogen sulfide given off may be recovered and can be recombined after oxidation to  $\text{SO}_2$  with the sodium carbonate solution to give sodium sulfite and set free carbon dioxide.

The recovery process above described is itself a new recovery process for the treatment of residual liquors of the character hereinbefore referred to for the production therefrom of further amounts of cooking liquors. It is of special value and application where sodium sulfide is present in the solution of the calcined or incinerated product and where sodium sulfide is not desired, or where a considerable reduction of the amount of sodium sulfide is desired, in a cooking liquor.

The process makes possible the elimination of the sodium sulfide by converting it into sodium carbonate and hydrogen sulfide, while the hydrogen sulfide may be burned to sulfur dioxide for further use in the process. In this way the objections incident to the presence of sodium sulfide in the cooking operation are overcome; while the process nevertheless makes possible the use of sodium sulfate or niter cake as a source of additional sodium and sulfur compounds in the process.

From one aspect the process may be considered to involve the conversion of sodium sulfate by reduction into sodium sulfide, the decomposition of the sodium sulfide with carbon dioxide to form a carbonate of sodium

and hydrogen sulfide, the burning of the hydrogen sulfide to form sulfur dioxide, and the use of the sulfur dioxide for treating sodium carbonate to form sodium sulfite and carbon dioxide. When the sodium sulfate is added to the residual liquor, these operations are combined with the other operations above described incident to the production of further amounts of cooking liquor from the residual liquor.

Owing to the formation of sodium carbonate during the calcining or incinerating operations, the amount of carbon dioxide formed by treating the sodium carbonate solution with sodium bisulfite will be in excess of that required for converting sodium sulfide into sodium carbonate. A part of this excess carbon dioxide may be used to convert sodium carbonate into sodium bicarbonate which may be precipitated in the carbonating tower or tank and recovered therefrom. The introduction of carbon dioxide into the solution of sodium carbonate and sodium sulfide may take place in an absorption tower with baffles or other filling material or obstructions to insure adequate absorption and reaction, or carbon dioxide can be introduced through a porous bottom, e. g., filtros bottom, into a tank of sufficient depth to insure adequate absorption of the carbon dioxide in the liquor.

Instead of using different apparatus for the carbonating operation and the sulfur dioxide absorption operation, these operations can advantageously be combined by using a deep tank of small cross section and introducing the sulfur dioxide at the bottom through a porous medium such as filtros plates. By introducing sulfur dioxide in this manner into a solution containing sodium carbonate and sodium sulfide, sodium sulfide will be decomposed and hydrogen sulfide driven off, while the sulfur dioxide will react upon the sodium carbonate in the lower part of the tank, setting free carbon dioxide which in its upward passage will react with the sodium sulfide to set free hydrogen sulfide. When operating in this way the hydrogen sulfide will be driven off first with a limited amount of carbon dioxide and the main portion of carbon dioxide will be subsequently removed. The hydrogen sulfide can be utilized as above described while the carbon dioxide can similarly be employed for further carbonating operations.

Other methods of decomposing the sodium sulfide or polysulfides and removing them from a solution of the melt can also be employed, although we consider the cyclic process above described as particularly advantageous. Where only small amounts of sulfide are present, they may be removed for example by adding iron sulfate, with resulting precipitation of iron sulfide. Where sodium carbonate is present, calcium sulfate

can be added to remove the carbon dioxide as calcium carbonate, leaving sodium sulfate in the solution, and sodium bisulfate can then be added to decompose the sulfides and drive off hydrogen sulfide. Further amounts of sodium sulfate can be added if desired and the solution then treated to convert the sodium sulfate into sodium sulfite, or into sodium sulfite with excess sulfur dioxide.

10 We have further found that when residual liquors of the character referred to are subjected to calcination without smelting, the solution or extract obtained from the calcined product may contain small amounts of sodium sulfide or polysulfides, particularly where the calcination is carried out under reducing conditions; and that the solutions so obtained can advantageously be treated in the same manner as solutions of smelted 15 products for the removal of sulfides therefrom. Thus, in case the residual liquor is evaporated and calcined or carbonized under reducing conditions, and then leached to extract the soluble salts therefrom, and a solution obtained which contains sodium sulfide, this solution can be treated first to convert the sodium sulfide into other compounds, in much the same manner that solutions of the smelted product are treated for the conversion 20 of the sodium sulfide into other products.

The invention will be further illustrated by the following specific examples.

Woods of varying kinds, such as spruce, hemlock or other long fiber woods, or hard 35 woods such as birches, beeches and maples, or chipped and screened, to give chips of approximately uniform size, (a good size being  $\frac{3}{8}$ " to  $\frac{5}{8}$ " along the grain) charged into a 40 digester, and cooked with a cooking liquor containing essentially normal sodium sulfite, as described in our prior application, U. S. Serial No. 481,147. By gradually and slowly heating the digester charge where necessary 45 and insuring a thorough penetration of the chips with the cooking liquor during the preliminary portion of the heating operation, (preferably below  $110^{\circ}$  C.) the digester can subsequently be heated to a higher temperature 50 and pressure without objectionable action upon the chips, and with substantially complete cooking of the chips even when long fibered resinous woods are employed. The cooking operation can be carried out as a single stage operation, or in successive stages, and, where two stages are employed, a different cooking liquor can be used in the second stage. When a normal sodium sulfite cooking liquor is used in the first stage, sodium sulfide 55 may be present in the second stage with less objections than are incident to its use in the sulfate process.

The residual liquor from the normal sodium sulfite cooks above referred to can be directly treated for the recovery of fresh

cooking liquors therefrom, or a part of the residual liquor can be returned without treatment for use in making up the charge for further cooking operations, in which case the cooking liquor will be a mixture of residual liquor and fresh sodium sulfite liquor which may be that obtained by the regenerative process.

The residual liquor from the cooking process in which sodium sulfite and caustic soda are employed, or from the process in which sodium sulfite and excess sulfur dioxide are employed, can similarly be treated directly for the recovery of fresh cooking liquors therefrom or a part of the residual liquor can be returned without treatment for use in making up the charge of further cooking operations, in which case the cooking liquor will be of a composite character, being made up in part of residual liquor and in part of fresh cooking liquor obtained by the regenerative process of the present invention. By returning part of the residual liquor and reusing it, the content of the residual liquor in organic material and inorganic constituents can be built up so that a more concentrated liquor is available for further treatment in the regeneration process, and we claim such operations as part of our invention.

The residual liquor may be evaporated in a multiple effect evaporator such as a triple effect Yaryan evaporator to about  $36^{\circ}$  to  $38^{\circ}$  Bé. and then run through a rotary furnace and converted into a product which may be referred to as green ash. This green ash may then be fed into the preheated smelter and burned and smelted to form a free running melt which is conveyed to the dissolving tank. The green ash was found to contain a sufficient amount of organic matter to burn readily without additional fuel, and the burning and melting operations appear more advantageous than those of the sulfate process. The calcination of the concentrated liquor in rotary furnaces also appeared to take place with less flame than appears in the sulfate process, so that a greater percentage of total heat units is retained in the green ash when discharged from the rotary to be charged into the smelter. The ease of burning of the ash and the low melting point of the smelted product was found to enable the smelting operation to take place in a particularly advantageous manner.

When the liquor in the dissolving tank, into which the hot melt was received had reached a density of about  $26^{\circ}$  Bé, hot the liquor was found on analysis to contain considerable carbonate, some sulfides and a considerable amount of sulfite. When this liquor was treated with hydrochloric acid, considerable sulfur was thrown out of solution. When treated with sodium bisulfite solution little sulfur was thrown out of solution, al-

though the liquor was made acid to phenolphthalein.

Instead of using fresh water or wash water to dissolve the melt, or to leach the calcined unsmelted product, the residual liquor from the process can be used for this purpose, thus building up the strength of the liquor and saving in evaporation. Where the residual liquor contains considerable unconsumed sodium sulfite, this excess of reagent will be made available in further cooking operations. By dissolving the melt in the fresh residual liquor, and by then removing the hydrogen sulfide and so treating the resulting solution with sulfur dioxide as to convert the carbonate into sulfite, and by clarifying if necessary to remove precipitated material, etc., a suitably concentrated cooking liquor can be obtained well adapted for reuse in the cooking step of the process.

Instead of treating residual liquors from the normal sodium sulfite cooking process, the residual liquor from the process in which caustic soda and sodium sulfite are employed can be treated in a similar way. In this case, however, the residual liquor will be of a somewhat different composition, and, in order to regenerate a similar cooking liquor, causticizing of some of the sodium carbonate with lime can replace the conversion of a corresponding amount of sodium carbonate to sodium sulfites may be used, and the residual liquor by evaporation, calcination, smelting and dissolving, can be carried out in a similar manner to that above described with the normal sodium sulfite residual liquors. To the extent that the resulting solution of the melt is required to be converted into sodium sulfite, similar methods to those above described can be used, supplemented by causticizing of part of the liquor with lime to convert sodium carbonate into caustic soda.

Residual liquors from the pulp making process in which acid sodium sulfite, or sodium sulfite with excess sulfur dioxide (as hereinbefore defined), are used, can also be treated in a somewhat similar way for the regeneration of cooking liquor therefrom. In this case, however, the residual liquor will be of a somewhat different composition and the treatment may be modified. The acid character of the residual liquor, and the increased content of sulfur dioxide in proportion to the sodium content tends to cause an increased amount of the sulfur dioxide to be given off during the concentrating, calcining and smelting operations. This sulfur dioxide can be recovered, however, e. g., by absorption and returned to the process. The residual liquor can also be advantageously treated to neutralize it before it is subjected to the concentrating, carbonizing and smelting operation. For this purpose the solution of the melt, or the partially causticized solution of the melt, may be used. By add-

ing the desired amount of the melt directly to such a residual liquor, the liquor will serve to dissolve the melt and will be preheated and neutralized to a greater or less extent at the same time. The neutralized residual liquor, neutralized in this or some other suitable manner, may then be subjected to evaporation, carbonization and smelting in the same general manner previously described. The solution of the melt thus obtained can also be treated in the same general manner previously described, but in order to provide a sufficient excess of sulfur dioxide, a correspondingly increased amount should be added. This can readily be supplied in the form of gases from a sulfur burner and in part by sulfur dioxide resulting from the burning of hydrogen sulfide given off in the process itself, in the manner hereinbefore referred to.

It will thus be seen that the present invention provides improved methods of regenerating the residual liquors from processes in which normal sodium sulfite, or sodium sulfite and caustic soda, or sodium sulfite and sodium bisulfite, or sodium sulfite and sulfuric acid, etc. are employed, for the production of further amounts of cooking liquor therefrom; and that the operations can in this way be improved and regulated and controlled in a particularly advantageous manner. Among the various features of advantage which the invention presents, as hereinbefore described, are included the reutilization of residual liquor itself in further cooking operations either with or without admixture of fresh amounts of reagents thereto; the recovery of the chemicals contained in the residual liquor by various methods of procedure whereby they are made available for further cooking operations; the evaporation of the residual liquors, carbonization and smelting, and dissolving of the melt with subsequent treatment of the resulting solution for the regeneration of cooking liquor therefrom; the carbonization of the concentrated residual liquor without excessive reduction and resulting recovery from the carbonized product of soda for further use in the process; the utilization of existing equipment of sulfate mills with a moderate amount of change and expense, and with advantages hereinbefore described, and with avoidance of certain objections incident to the sulfate process itself; the utilization of sodium sulfate or niter cake in supplying additional chemicals to the process, with elimination of sulfide radical if desired and utilization of the sulfur content thereof in the further carrying on of the process; the treatment of solutions containing sodium sulfide to remove sulfur therefrom and convert the sodium into sodium sulfite, with utilization of the hydrogen sulfide given off for producing sulfur dioxide

by combustion; and various other features of improvement hereinbefore described.

The improvements of the present invention supplement the improvements of our 5 prior applications and are of value in connection with manufacture of pulp and paper from woods of various kinds, including not only woods commonly considered as pulp woods such as spruce and poplar, but also 10 woods which are not commonly considered as pulp woods at all, or woods which are considered of little value for pulp making purposes, such as the heavy hard woods (birches, beeches, maples, oaks, gums, etc.) and resinous 15 coniferous or long fibered woods such as jack-pine, loblolly pine, tamarack, etc.

While the invention has been described more particularly in connection with the use of sulfites of sodium, yet it will be understood that sulfites of potassium or mixtures of sulfites of sodium and potassium can be similarly used; and that sulfites of magnesium can to some extent likewise be used, although we consider the use of sodium sulfites as particularly advantageous. Sulfites of potassium will ordinarily be too expensive for commercial use, although they may be used where cheap deposits containing suitable potassium compounds are available. 30 Similarly, mixtures of magnesium and sodium sulfites may be used, and the residual liquors from their use treated for the regeneration of further amounts of cooking liquor therefrom.

35 Magnesium sulfate, either alone or accompanied by sodium sulfate, may be added to a solution of the melt to convert the sodium carbonate into sodium sulfate and the magnesium sulfate into magnesium carbonate. 40 The sodium sulfide may be eliminated by precipitation or by volatilization of the sulfide radicle. For example, iron sulfate can be used for precipitation of iron sulfide, or sulfuric acid, nitre cake, or  $\text{CO}_2$  may be used to 45 drive off  $\text{H}_2\text{S}$ . The sodium sulfate solution can then be treated with  $\text{CaSO}_4$  and  $\text{H}_2\text{SO}_4$  to form  $\text{CaSO}_4 \cdot 2\text{H}_2\text{O}$  and leave an acid solution containing sodium sulfite. Other soluble metallic salts may be used to precipitate 50 insoluble metallic sulfides, e. g. copper sulfate.

We claim:

1. In the treatment of residual liquors from pulp-making operations in which an 55 alkali metal sulfite is employed in the cooking liquor, the improvement which comprises evaporating such liquors, subjecting the residue to calcination, smelting the calcined product, dissolving the resulting melt and 60 treating the solution to decompose sulfide contained therein.

2. In the treatment of residual liquors from pulp-making operations in which an alkali metal sulfite is employed in the cooking 65 liquor, the improvement which comprises

evaporating such liquor, subjecting the residue to calcination, smelting the calcined product, dissolving the resulting melt and treating the solution to decompose sulfide contained therein, said treatment including the treatment of the solution with carbon dioxide to convert sulfide into a carbonate and to drive off hydrogen sulfide. 70

3. In the treatment of residual liquors from pulp-making operations in which an alkali metal sulfite is employed in the cooking liquor, the improvement which comprises subjecting such residual liquors to evaporation, subjecting the residue to calcination, and subjecting the calcined product to a smelting 80 operation.

4. In the treatment of residual liquors from pulp-making operations in which a sodium sulfite is employed in the cooking liquor, the improvement which comprises evaporating such residual liquors, subjecting the residue to calcination, and subjecting the calcined product to a smelting 85 operation.

5. The further improvement in the process of claim 4 in which the melt is dissolved and the resulting solution treated with an acid substance to decompose sulfide present in the liquor. 90

6. The further improvement in the process of claim 4 in which the melt is dissolved and the resulting solution treated for the production of further amounts of cooking liquor therefrom. 95

7. The further improvement in the process of claim 4 in which the melt is dissolved in a portion of the residual liquor and the resulting solution treated for the production of further amounts of cooking liquor therefrom. 100

8. The improvement in the process of claim 4 in which the melt is dissolved to form a solution, the solution treated with carbonic acid radical to decompose sodium sulfide and drive off hydrogen sulfide, the hydrogen sulfide burned to sulfur dioxide and sulfur dioxide absorbed in the solution from which the hydrogen sulfide has been driven off. 105

9. The improvement in the process of claim 4 which comprises dissolving the melt to form a solution thereof, treating the solution with carbon dioxide to decompose sodium sulfide and drive off hydrogen sulfide, burning the hydrogen sulfide and some sulfur for the production of sulfur dioxide, and treating the solution of the melt from which the hydrogen sulfide has been driven off with sulfurous acid radical to convert the carbonate into a sulfite. 115

10. The improvement in the treatment of residual liquors from pulp-making operations in which a sulfite of sodium is employed in the cooking liquor, which comprises evaporating the residual liquor, calcining and smelting the residual material, dissolving the melt to form a solution thereof, treating 120

130

the solution with carbon dioxide to decompose sodium sulfide and drive off hydrogen sulfide, treating the resulting solution with an acid sulfite solution containing sufficient sulfur dioxide to convert the carbonate to sulfite, burning sulfur and the hydrogen sulfide to form sulfur dioxide, absorbing sulfur dioxide to form a further amount of acid sulfite solution, and employing such acid sulfite solution for treating the solution of the melt in the earlier step of the process.

11. The improvement in the claim 10 in which additional sulfate of sodium is added prior to the smelting operation, thereby giving an increased amount of sodium compounds in the solution of the melt and an increased amount of sodium sulfide and of hydrogen sulfide in the process.

12. The method of producing solutions containing sodium sulfite from a sodium sulfate which comprises reducing sodium sulfate to sodium sulfide, treating a solution containing the sodium sulfide with carbon dioxide to form a sodium carbonate and hydrogen sulfide, and absorbing sulfur dioxide in the sodium carbonate solution to form sodium sulfite.

13. in the treatment of residual liquors from pulp-making operations in which a sulfite of sodium is employed, and in which the residual liquor is concentrated, the residue calcined and the product leached to form a solution containing sodium carbonate and sodium sulfide, the step which comprises treating such solution with carbon dioxide to convert the sulfide into carbonate and set free hydrogen sulfide, and the further step which comprises treating the solution so obtained with the sulfurous acid radical to convert carbonate into sulfite.

14. The cyclic process of forming solutions containing sodium sulfite from solutions containing sodium carbonate, which comprises treating such carbonate solutions with acid sodium sulfite to convert the carbonate into sulfite, absorbing sulfur dioxide in part or all of the sulfite solution so formed, and treating a further amount of carbonate solution therewith.

15. The cyclic process of forming solutions containing sodium sulfite from solutions containing sodium carbonate and sodium sulfide, which comprises subjecting such solutions to treatment with carbon dioxide to convert sulfide into carbonate and set free hydrogen sulfide, burning the hydrogen sulfide together with some sulfur to form sulfur dioxide, absorbing the sulfur dioxide in the carbonate solution to set free carbon dioxide, and using the carbon dioxide in the further carrying out of the carbonating step of the process for converting sulfide into carbonate.

16. The cyclic process of forming solutions containing sodium sulfite from solutions containing sodium carbonate and sodium sulfide,

which comprises subjecting such solutions to treatment with carbon dioxide to convert sulfide into carbonate and set free hydrogen sulfide, burning the hydrogen sulfide together with some sulfur to form sulfur dioxide, absorbing the sulfur dioxide in a sodium sulfite solution to form an acid sulfite solution, treating the carbonate solution with the acid sulfite solution to convert the carbonate into sulfite, and using the carbon dioxide set free for the further carrying out of the carbonating step of the process.

17. In the treatment of residual liquors from the cooking of cellulose-bearing material with a cooking liquor containing sodium sulfite, which residual liquors have been concentrated and the residue calcined, and the product treated to form a solution containing sodium salts, the step which comprises treating such solution with carbon dioxide and subsequently with sulfur dioxide.

18. In the treatment of residual liquors from pulp-making operations in which a sulfite of a strong base is employed in the cooking liquor, the improvement which comprises evaporating such liquors, subjecting the residue to calcination, smelting the calcined product, dissolving the melt in a portion of the residual liquor and treating the resulting solution for the production of further amounts of cooking liquor therefrom.

19. The method of treating solutions containing sodium sulfide and sodium carbonate, which comprises treating such solution with carbon dioxide to decompose sulfide of sodium and form sodium carbonate in which a relatively pure carbon dioxide is used to treat the solution, thereby giving hydrogen sulfide, burning the hydrogen sulfide to form sulfur dioxide and absorbing sulfur dioxide in the solution.

20. The method of treating solutions containing sodium sulfide and sodium carbonate, which comprises treating such solution with carbon dioxide to decompose sulfide of sodium and form sodium carbonate, burning the hydrogen sulfide and some sulfur to form sulfur dioxide, absorbing sulfur dioxide in a solution containing sodium sulfite, to give an acid solution of sodium sulfite, and treating the solution containing sodium carbonate with such acid sulfite solution.

21. The method of treating solutions containing sodium sulfide and sodium carbonate, which comprises treating such solution with carbon dioxide to decompose sulfide of sodium and form sodium carbonate, burning the hydrogen sulfide and some sulfur to form sulfur dioxide, absorbing sulfur dioxide in a solution containing sodium sulfite, to give an acid solution of sodium sulfite, and treating the solution containing sodium carbonate with such acid sulfite solution in which the carbon dioxide obtained in a relatively pure and concentrated state is used to the required

extent to treat the solution containing sodium sulfide and sodium carbonate to decompose sodium sulfide and set free hydrogen sulfide therefrom.

5. 22. The method of treating solutions containing sodium sulfide and sodium carbonate, which comprises treating such solution with carbon dioxide to decompose sulfide of sodium and form sodium carbonate, treating the solution, after removing hydrogen sulfide therefrom, with sulfurous acid radical to convert sodium carbonate to the desired extent into a sulfite of sodium.

15. 23. The method of treating solutions containing sodium sulfide and sodium carbonate, which comprises treating such solution with carbon dioxide to decompose sulfide of sodium and form sodium carbonate, treating the carbonate solution, after the removal of hydrogen sulfide, with an acid solution of sodium sulfite containing an excess of sulfur dioxide, thereby obtaining a solution of sodium sulfite for use in further cooking operation.

25. 24. The method of treating solutions containing sodium sulfide and sodium carbonate, which comprises treating such solution with carbon dioxide to decompose sulfide of sodium and form sodium carbonate, treating the carbonated solution, after driving off hydrogen sulfide, with an acid solution of sodium sulfite containing excess sulfur dioxide to convert the carbonate into a sulfite, absorbing sulfur dioxide in the resulting sodium sulfite solution or in a portion of it and thereby forming a further amount of acid sulfite solution, and treating further amounts of carbonated solution with such acid solution.

35. 25. A cyclic process which comprises digesting raw cellulosic material in a sulphurous acid solution of a soluble alkali or alkaline earth sulphite, neutralizing the spent liquor resulting from such digestion, separating the pulp from such neutralized spent liquor, burning the combustible content and smelting the inorganic mineral content of such spent liquor in a reducing atmosphere in a manner to produce sulphide and carbonate, recovering the inorganic smelt in water, carbonating the smelt solution, and acidifying the carbonated solution with sulphur dioxide in a manner to produce fresh acid digesting liquor.

45. 26. A cyclic process which comprises digesting raw cellulosic material in a sulphurous acid solution of a soluble alkali or alkaline earth sulphite, neutralizing the spent liquor resulting from such digestion, separating the pulp from such neutralized and spent liquor, burning the combustible and smelting inorganic material content of such liquor in a reducing atmosphere in a manner to produce sulphide and carbonate, recovering the inorganic smelt in water, carbonating the smelt solution, employing a por-

tion of such carbonate solution together with cyclic make-up compounds for such neutralization, and acidifying the remainder of the carbonated solution with sulphur dioxide in a manner to produce a fresh acid digesting liquor.

5. 27. A process which comprises concentrating and burning the combustible content and smelting the inorganic content of spent liquor resulting from the digestion of raw cellulosic material in a sulphurous acid solution of soluble alkali sulphite or alkaline earth sulphite, in a manner to produce substantially only sulphide and carbonate, recovering the smelted inorganic compounds in water, carbonating the smelt solution with substantially pure carbon dioxide and controlling such carbonation to produce a substantially pure hydrogen sulphide, burning such hydrogen sulphide and recovering the products of combustion, acidifying the carbonated solution with a substantially pure sulphur dioxide, controlling such acidification to produce a substantially pure carbon dioxide, and utilizing such carbon dioxide in the carbonation of other smelt solution.

25. 28. A process which comprises concentrating and burning the combustible content and smelting the inorganic content of spent liquor resulting from the digestion of raw cellulosic material in a sulphurous acid solution of soluble alkali sulphite or alkaline earth sulphite, in a manner to produce substantially only sulphide and carbonate, recovering the smelted inorganic compounds in water, carbonating the smelt solution with substantially pure carbon dioxide and controlling such carbonation to produce a substantially pure hydrogen sulphide, acidifying the carbonated solution with a substantially pure sulphur dioxide, controlling such acidification to produce a substantially pure carbon dioxide, and utilizing such carbon dioxide in the carbonation of other smelt solution.

5. 29. A process which comprises concentrating and burning the combustible content and smelting the inorganic content of spent liquor resulting from the digestion of raw cellulosic material in a sulphurous acid solution of a soluble alkali and alkaline earth sulphite, in a reducing atmosphere in a manner to produce substantially only sulphide and carbonate, recovering the smelted inorganic compounds in water, carbonating the smelt solution, oxidizing any remaining sulphide, and acidifying the carbonated solution with sulphur dioxide in such amount as is needed to produce a fresh acid digesting liquor.

25. 30. A process which comprises digesting raw cellulosic material in a sulphurous acid solution of a soluble alkali sulphite or alkaline earth sulphite, concentrating and burning the combustible content and smelting

- the inorganic content of spent liquor resulting from such digestion in a manner to produce sulphide and carbonate, recovering the smelted inorganic compounds in water, carbonating the smelt solution with carbon dioxide and controlling such carbonation to produce hydrogen sulphide and to effect a conversion of substantially all the sulphide to carbonate, burning such hydrogen sulphide to produce sulphur dioxide, recovering the gaseous products of combustion, acidifying the carbonated solution with sulphur dioxide and controlling such acidification to produce a substantially pure carbon dioxide and a sulphite solution, utilizing the carbon dioxide obtained in such acidification for the carbonation of other smelt solution, and utilizing said products of combustion in the production of a sulphite cooking liquor.
31. A process which comprises digesting raw cellulosic material in a sulphurous acid solution of a soluble alkali sulphite or alkaline earth sulphite, concentrating and burning the combustible content and smelting the inorganic content of spent liquor resulting from such digestion in a manner to produce sulphide and carbonate; recovering the smelted inorganic compounds in water, carbonating the smelt solution with a strong carbon dioxide, burning the hydrogen sulphide resulting from such carbonation and recovering the sulphur dioxide thereby produced, acidifying the carbonated solution with digester relief gas, recovering and utilizing the carbon dioxide liberated in such acidification for the carbonation of other like smelt solution, and utilizing the products of combustion of the hydrogen sulphide in the production of fresh cooking liquor.
32. A process which comprises digesting raw cellulosic material in a sulphurous acid solution of a soluble alkali sulphite or alkaline earth sulphite, concentrating and burning the combustible content and smelting the inorganic content of spent liquor resulting from such digestion in a manner to produce sulphide and carbonate, recovering the smelted inorganic compounds in water, carbonating the smelt solution with carbon dioxide, burning the hydrogen sulphide resulting from such carbonation and recovering the sulphur dioxide thereby produced, acidifying the carbonated solution with digester relief gas, recovering and utilizing the carbon dioxide liberated in such acidification for the carbonation of other smelt solution, treating said carbonated solution with sulphur burner gas and the products of combustion of said hydrogen sulphide, and finally adding relief gas thereto to produce a fresh acid cooking liquor having a high free  $\text{SO}_2$  content.
33. A process which comprises digesting raw cellulosic material in a sulphurous acid solution of a soluble alkali or alkaline earth sulphite, recovering sulphur dioxide from the acid spent liquor resulting from such digestion, concentrating and burning the combustible content and smelting the inorganic content of such spent liquor in a manner to produce sulphide and carbonate, recovering the smelted inorganic compounds in water, carbonating the smelt solution, burning the hydrogen sulphide resulting from such carbonation and recovering the sulphur dioxide thereby produced, acidifying the carbonated solution with digester relief gas, utilizing the carbon dioxide liberated in such acidification for the carbonation of other smelt solution, and further treating said acidified solution with sulphur burner gas, the products of combustion of the hydrogen sulphide, and the sulphur dioxide recovered from the acid spent liquor.
34. A cyclic process which comprises concentrating spent liquor resulting from the digestion of raw cellulosic material in a sulphurous acid solution of a soluble alkali sulphite or alkaline earth sulphite, smelting the inorganic content of such liquor in a reducing atmosphere to produce carbonate and sulphide, and recovering the latter in an aqueous solution, carbonating such solution with carbon dioxide and thereby producing a carbonate and hydrogen sulphide, acidifying said carbonated solution with sulphur dioxide, and recovering and reusing the recovered carbon dioxide resulting from such acidification in the aforesaid carbonation of the smelted and recovered sulphide.
35. That process which comprises smelting the mineral content of spent liquor, resulting from the digestion of raw cellulosic material in an alkaline sulphite or alkaline earth sulphite cooking liquor, to produce mineral sulphide and mineral carbonate, recovering such sulphide and carbonate in an aqueous solution, treating such solution with carbon dioxide to carbonate the mineral sulphide, treating the resulting solution with sulphur dioxide to produce a sulphite liquor, recovering carbon dioxide resulting from such acidification, and using such recovered carbon dioxide for the aforesaid carbonation.
36. That process which comprises smelting the mineral content of spent liquor, resulting from the digestion of raw cellulosic material in an alkaline sulphite or alkaline earth sulphite cooking liquor, to produce mineral sulphide and mineral carbonate, recovering such sulphide and carbonate in an aqueous solution, treating such solution with carbon dioxide to carbonate the mineral sulphide, treating the resulting solution with sulphur dioxide to produce a sulphite liquor, recovering hydrogen sulphide from such carbonation, and burning the same to produce sulphur dioxide, recovering carbon dioxide resulting from such acidification, using such

recovered carbon dioxide for the aforesaid carbonation, and recovering and using such last mentioned sulphur dioxide in the acidification of said sulphite liquor.

- 5 37. A process for recovering and utilizing the products produced in recovering the base compound from spent sulphite liquors in forming a fresh sulphite cooking liquor, which comprises treating a carbonate solution with sulphur dioxide to convert it to a normal sulphite solution, recovering the carbon dioxide arising from such treatment and carbonating therewith a sulphite smelt solution comprising sulphide to a carbonate 70 solution, thereby liberating hydrogen sulphide, recovering and burning such hydrogen sulphide to sulphur dioxide, and acidifying the normal sulphite solution with the recovered sulphur dioxide.
- 10 38. A process which comprises cooking raw cellulosic material in an alkaline solution of sodium sulphite; separating the pulp from the spent cooking liquor; smelting the inorganic mineral content and burning the combustible content of such spent liquor, recovering the inorganic smelted compounds; and passing the products of combustion from such smelting operation in contact with like spent liquor, for the recovery of the soluble 25 content of such products of combustion.

30 39. The cyclic process for producing pulp from wood which comprises cooking wood in an acid liquor containing a sulfite of an alkali, separating a residual liquor from the resulting fibrous material, drying the residual liquor, carbonizing organic constituents of the liquor, dissolving from the resulting product soluble compounds including alkali carbonate and alkali sulfide, subjecting the dissolved compounds to a regulated oxidizing treatment to convert the sulfide into sulfite under conditions to substantially prevent the formation of alkali thiosulfate, acidifying the resulting sulfite solution to produce a cooking liquor substantially free from thiosulfate, and cooking more wood with said liquor.

35 40. The cyclic process for producing pulp from wood which comprises cooking wood in a liquor containing a sulfur compound of an alkali, separating the residual liquor from the resulting fibrous material, drying the residual liquor, burning dried carbonaceous constituents of the liquor, dissolving from the resulting ash soluble compounds including alkali sulfide and alkali carbonate, subjecting the alkali sulfide to a treatment to remove the sulfide-sulfur, oxidizing it to form sulfur dioxide, and recombining the sulfur dioxide so formed with the alkali compounds; forming a cooking liquor from the resulting sulfite solution, and cooking more wood with said liquor.

45 41. A process which comprises cooking raw cellulosic material in an alkaline solu-

tion of sodium sulfite; separating the pulp from the spent cooking liquor; smelting the inorganic mineral content and burning the combustible content of such spent liquor in a reducing atmosphere to produce sodium sulfide; and recovering the inorganic compounds for reuse in the cooking of other cellulosic material.

42. A process which comprises cooking raw cellulosic material in an alkaline cooking liquor containing sodium sulfite; separating the pulp from the spent cooking liquor; burning the combustible content and smelting the inorganic mineral content of such spent liquor in a reducing atmosphere to form 80 sodium sulfide; recovering the sodium sulfide in water; carbonating the sodium sulfide of the solution to sodium carbonate; and acidifying the carbonate solution with sulfur dioxide.

43. A process which comprises cooking raw cellulosic material in an alkaline solution of sodium sulfite; separating the pulp from the spent cooking liquor; burning the combustible content and smelting the inorganic 90 mineral content of such spent liquor in a reducing atmosphere in a manner to produce sodium sulfide and sodium carbonate; carbonating the sodium sulfide of the smelt solution to sodium carbonate; acidifying the 95 whole sodium carbonate solution with sulphur dioxide to convert said sodium carbonate to sodium sulfite; and recovering and utilizing the carbon dioxide liberated in such acidification in the carbonation of other 100 smelt liquor.

44. A process which comprises cooking raw cellulosic material in an alkaline solution of sodium sulphite; separating the pulp from the spent cooking liquor; burning the combustible content and smelting the inorganic mineral content of such spent liquor in a reducing atmosphere in a manner to produce sodium sulphide and sodium carbonate; carbonating the smelt solution; and 110 recovering the sulphur to the hydrogen sulphide liberated in such carbonation in the form of a sodium salt.

45. A process which comprises cooking raw cellulosic material in an alkaline solution 115 of sodium sulphite; separating the pulp from the spent cooking liquor; burning the combustible content and smelting the inorganic mineral content of such spent liquor in a reducing atmosphere in a manner to produce sodium sulphide and sodium carbonate; carbonating the smelt solution; recovering and burning the hydrogen sulphide liberated in such carbonation to sulphur dioxide; and recovering the sulphur dioxide in the form 120 of sodium sulphite.

46. A process which comprises cooking raw cellulosic material in an alkaline solution of sodium sulphite; separating the pulp from the spent cooking liquor; burning the com- 130

bustible content and smelting the inorganic mineral content of such spent liquor in a reducing atmosphere in a manner to produce sodium sulphide and sodium carbonate; carbonating the smelt solution; and recovering the sulphur of the hydrogen sulphide liberated in such carbonation in the form of sodium sulphite.

47. A process which comprises concentrating and burning the combustible content and smelting the inorganic content of spent liquor resulting from the digestion of raw cellulosic material in an alkaline solution of sodium sulphite in a manner to produce sodium sulphide and sodium carbonate; recovering the smelted inorganic compounds in water; carbonating the smelt solution; recovering the sulphur of the hydrogen sulphide liberated in such carbonation in the form of a sodium salt; acidifying the carbonate solution with sulphurous acid; and recovering and utilizing the carbon dioxide liberated in such acidification in the carbonation of other smelt liquor.

48. A process which comprises concentrating and burning the combustible content and smelting the inorganic mineral content of spent liquor resulting from the digestion of raw cellulosic material in an alkaline solution of sodium sulphite in a manner to produce sodium sulphide and sodium carbonate; recovering the smelted inorganic compounds in water; carbonating the smelt solution; recovering the sulphur of the hydrogen sulphide liberated in such carbonation in the form of a sodium-sulphur compound; acidifying the carbonate solution with sulphur dioxide; and recovering and utilizing the carbon dioxide liberated in such acidification in the carbonation of other smelt liquor.

49. A process which comprises concentrating and burning the combustible content and smelting the inorganic mineral content of spent liquor resulting from the digestion of raw cellulosic material in an alkaline solution of sodium sulphite in a manner to produce sodium sulphide and sodium carbonate; recovering the smelted inorganic compounds in water; carbonating the smelt solution with substantially pure carbon dioxide and controlling such carbonation to produce substantially pure hydrogen sulphide; recovering and burning such hydrogen sulphide and recovering the products of combustion; acidifying the carbonate solution with a sulphurous acid solution formed in part from said recovered sulphur dioxide and the products of combustion of sulphur-bearing material; controlling such acidification to yield a substantially pure carbon dioxide; and recovering and utilizing such carbon dioxide in the carbonation of other smelt liquor.

50. A process which comprises concentrating and burning the combustible content and smelting the inorganic mineral content of

spent liquor resulting from the digestion of raw cellulosic material in an alkaline solution of sodium sulphite in a manner to produce sodium sulphide and sodium carbonate; recovering the smelted inorganic compounds in water; carbonating the smelt solution with substantially pure carbon dioxide and controlling such carbonation to produce substantially pure hydrogen sulphide; recovering the sulphur of the hydrogen sulphide liberated in such carbonation in the form of a sodium salt; acidifying the carbonate solution with sulphurous acid formed from the products of combustion of sulphur-bearing material; controlling such acidification to produce a substantially pure carbon dioxide; and recovering and utilizing such carbon dioxide in the carbonation of other smelt liquor.

51. A process which comprises concentrating and burning the combustible content and smelting the inorganic content of spent liquor resulting from the digestion of raw cellulosic material in an alkaline liquor containing sodium sulphite in a manner to produce sodium sulphide and sodium carbonate; recovering the smelted inorganic compounds in water; carbonating the smelt solution with substantially pure carbon dioxide; and controlling such carbonation to produce substantially pure hydrogen sulphide; recovering such hydrogen sulphide; acidifying the carbonated solution with substantially pure sulphur dioxide to convert the sodium carbonate to sodium sulphite; controlling such acidification to produce a substantially pure carbon dioxide; utilizing such carbon dioxide in the carbonation of other smelt solution; treating a sodium compound employed for making up losses in the cycle for the production of sodium sulphide; utilizing the latter in producing a cooking liquor comprising sodium sulphite and sodium sulphide; and employing such cooking liquor for the digestion of other raw cellulosic material.

52. A process which comprises digesting raw cellulosic material in an alkaline liquor containing sodium sulphite; concentrating and burning the combustible content and smelting the inorganic content of spent liquor resulting from such digestion in a manner to produce sodium sulphide and sodium carbonate; recovering the inorganic smelted compounds in water; carbonating the smelt solution with carbon dioxide and controlling such carbonation to produce substantially pure hydrogen sulphide and to effect a conversion of substantially all the sodium sulphide to sodium carbonate; recovering the sulphur of such hydrogen sulphide in the form of a sodium salt; acidifying the sodium carbonate solution with sulphur dioxide and controlling such acidification to produce a substantially pure carbon dioxide and a sodium sulphite solution, and utilizing the carbon dioxide obtained in such

acidification for the carbonation of other smelt solution.

53. A process which comprises digesting raw cellulosic material in an alkaline cooking liquor containing sodium sulphite in solution; separating the pulp from the spent cooking liquor; smelting the inorganic mineral content and burning the combustible content of such spent liquor in a manner to 10 produce sodium sulphide and sodium carbonate; recovering the smelted inorganic compounds in water; carbonating the smelt solution with carbon dioxide; acidifying the carbonate solution with sulphur dioxide to 15 produce a solution of sodium sulphite; recovering the hydrogen sulphide liberated in such treatment in the form of a sodium salt; and adding sodium constituents to one of the liquors of the cycle in the form of an alkaline 20 sodium compound for making up losses in the cycle.

54. A process which comprises cooking raw cellulosic material in an alkaline solution of sodium sulphite and sodium sulphide; 25 separating the pulp from the spent cooking liquor; smelting the inorganic mineral content and burning the combustible content of such spent liquor in a reducing atmosphere to produce sodium sulphide; and recovering 30 the inorganic smelted compounds for reuse in the cooking of other cellulosic material.

55. A process which comprises cooking raw cellulosic material in an alkaline cooking liquor containing sodium-sulphur compounds; separating the pulp from the spent 35 cooking liquor; burning the combustible content and smelting the inorganic mineral content of such spent liquor in a reducing atmosphere to form sodium sulphide; recovering 40 the sodium sulphide in water; carbonating the sodium sulphide of the solution to sodium carbonate; and acidifying the carbonate solution with sulphur dioxide.

In testimony whereof we affix our signatures.

LINN BRADLEY.  
EDWARD P. McKEEFE.